

**1**

3,413,105

**GASOLINE ADDITIVE**

Curtis P. Parsons and Charles T. Pumpelly, Midland, Mich., assignors to The Dow Chemical Company, Midland, Mich., a corporation of Delaware  
No Drawing. Filed Jan. 3, 1966, Ser. No. 517,898  
2 Claims. (Cl. 44—72)

This invention relates to new gasoline fuel compositions containing a new additive which reduces the emission of hydrocarbons in the exhaust of internal combustion engines operating on the fuel.

Atmospheric contamination by automobile exhaust is a great and growing problem toward the control of which increased attention is being directed.

Additives such as alcohol, diethyl ether and nitromethane have been added to gasoline for various reasons and many of them produce a reduction in the hydrocarbon content of the exhaust. This reduction, however, is little if any more than can be accounted for by the oxygen in the additive, i.e., these additives merely serve as an expensive source of oxygen, and the same reduction in hydrocarbon content of the exhaust can equally well be attained by merely adjusting the carburetor to provide a leaner fuel mixture (higher air-to-fuel ratio). While such leaner fuel mixtures reduce the hydrocarbon content of the exhaust, they are objectionable for other reasons, such as excessive rate and temperature of combustion, burning of valves, etc.

According to the invention, the addition to gasoline of a small proportion of dibromofluoronitromethane (referred to hereinafter as DFN) substantially reduces the hydrocarbon emission of engines using the improved fuel, this improvement being far greater than would be expected the "leaning" effect of the oxygen contained in the additive. Thus, the engine can be operated with a normally rich fuel mixture and yet emit an exhaust having the low hydrocarbon content characteristic of that produced with lean fuel mixtures.

The amount of DFN can be varied widely, depending

5

10

20  
2530  
35**2**

on the type of engine, exhaust requirements, and other factors. In general, a substantial improvement is noted with as little as 1% by volume, while larger amounts, up to 5% or more, may be used with good results.

The practice of the invention is illustrated by the following example.

An automotive engine was operated on a dynamometer at 1500 r.p.m. and 15 horsepower. Using a full boiling range automotive fuel, the exhaust gas analysis was obtained. Under the same conditions except with 3.3% (vol.) of DFN in the fuel, the test was repeated:

|                                | No additive | Additive |
|--------------------------------|-------------|----------|
| CO <sub>2</sub> (percent)..... | 11.1        | 11.4     |
| O <sub>2</sub> (percent).....  | 0.62        | 0.94     |
| N <sub>2</sub> (percent).....  | 82.8        | 80.6     |
| CO (percent).....              | 1.50        | Zero     |
| Hydrocarbons (p.p.m.).....     | 412         | 290      |

We claim:

1. A gasoline fuel composition for internal combustion engines containing a minor proportion, effective to reduce the hydrocarbon content of the exhaust of an internal combustion engine operated on said fuel, of dibromofluoronitromethane.

2. The composition of claim 1 wherein the proportion of dibromofluoronitromethane is 1-5% by volume.

**References Cited****UNITED STATES PATENTS**

|           |         |                    |         |
|-----------|---------|--------------------|---------|
| 2,274,666 | 3/1942  | Clarke et al. .... | 44—57   |
| 2,583,048 | 1/1952  | Hannum et al. .... | 44—72   |
| 2,838,387 | 6/1958  | Rudel ....         | 44—79   |
| 3,133,844 | 5/1964  | Royer et al. ....  | 149—89  |
| 3,159,686 | 12/1964 | Burk et al. ....   | 260—644 |

DANIEL E. WYMAN, *Primary Examiner.*

Y. H. SMITH, *Assistant Examiner.*